

March 9, 1937.

M. KLEIN ET AL

2,073,067

SYRINGE

Filed Nov. 14, 1936



Fig. 1.



Fig. 2.



Fig. 7.



Fig. 3.



Fig. 6.



Fig. 4.



Fig. 5.

INVENTORS  
Max Klein & George Grunberg

BY  
Paul Klein  
ATTORNEY

## UNITED STATES PATENT OFFICE

2,073,067

## SYRINGE

Max Klein and George Grunberg, New York, N. Y.

Application November 14, 1936, Serial No. 110,849

15 Claims. (Cl. 128—215)

This invention relates to syringes in general, and particularly to the kind known as hypodermic syringes, and especially to what may be termed "armored" hypodermic syringes.

5 One of the prime objects of this invention is the method whereby a glass syringe may be reinforced at its weakest points of structure, and wherein particularly the shoulder portion and the tip of the syringe is strengthened by a bi-metallic, 10 electro-deposited, fused-on and firmly secured armor, but wherein the extreme end of the tip presents a clean, all-glass contacting surface for the needle end of the hub adapted to be removably secured to the syringe tip, and wherein, 15 during or after the application of the armor, the syringe material is re-annealed.

A further object of this invention is the method whereby the metallic armor, applied to the shoulder and tip of a glass syringe, is immovably anchored onto the glass and is trimmed at its 20 edges by rolling against the glass, so as to assure perfect contact and proper limits for the edges of the armor.

A further object of this invention is to provide 25 an armored glass syringe wherein the glass of the syringe is doubly annealed and re-glazed at the exposed glass surfaces, whereby distortion, strains within the glass, and warping of the syringe is prevented.

30 A further object of this invention is to provide in a doubly annealed glass syringe an armor about the shoulder and the tip thereof, and wherein the armor is caused to interlock with the glass, so as to prevent possible disengagement 35 therefrom, and wherein the extreme edge of the armor surrounding the tip terminates at the glass edge thereof, and wherein the edge of the armor surrounding the shoulder terminates below the shoulder portion at the body of the syringe, and 40 wherein the armor consists of a relatively soft, primary or underlayer of metal, such as copper, and a relatively hard top or upper layer of metal, such as rhodium, whereby a bi-metallic armor of the desired properties is provided.

45 Another very important object of this invention is to provide an armor for a glass syringe, which not only provides the desired protection against undue breakage and positively interlocks with the glass body of the syringe tip, but which assures a perfect union between the tip and the needle hub, and which is superior in many other ways to similar devices and is most inexpensive in production, as compared with such devices.

The foregoing and still other objects and further advantages of this invention will become

more fully apparent from the ensuing description, in connection with the accompanying drawing, which latter form an essential part of this disclosure, but by no means are intended to restrict the same to the actual illustrations, and in which—

Fig. 1 is a side view of an armored syringe, partially in cross-section;

Fig. 2 is an end view thereof;

Fig. 3 is an enlarged detailed view of the 10 armored portion of the syringe;

Fig. 4 is a modified form of an armored syringe with a threaded end;

Fig. 5 is still another modification of an 15 armored syringe with a bayonet lock;

Fig. 6 is a cross-section through a needle hub adapted to fit the tip of the device shown in Fig. 5; and

Fig. 7 represents a section through a still further important modification of this invention.

Referring now to Figs. 1 and 3, numeral 10 denotes the cylindrical body of the syringe which is made of glass and which is formed at 11 into what is known as shoulder, from which latter extends tip 12, provided with a passage 12'. It will be noted particularly in Fig. 3 that the material between the cylindrical body of the syringe and the tip is considerably reduced in thickness, as indicated at 13. Thus, the shoulder portion constitutes the weakest point of the glass syringe. Inasmuch as the needle hub has to be frequently attached to and removed from the tip of the syringe, the shoulder and the tip are subjected to great strains, due to which these parts usually break. It is this undesirable disadvantage which the present invention is intended to overcome. For accomplishing this purpose, an armor A is formed directly upon the glass around the shoulder and the tip, and extends from the extreme upper tip edge, at 14, to somewhat below the shoulder, at 15, and engages a portion of the body of the syringe.

The manufacture of glass syringes is a well known art. After the product is finished, it is annealed in order to remove strains and stresses within the glass. The armor of the present invention is applied to the thus annealed syringe structure in the following manner:

The surface of the glass portions to which the armor is to be applied and which are normally glazed, are roughened by grinding, etching or otherwise, so as to prepare it for the reception of an electrolytic deposit, first, of a soft underlayer, such as copper, which latter serves as depositing base for a hard upper metal layer, such

15

20

25

30

35

40

45

50

55

as rhodium, which is superimposed upon the copper. The hub of a hypodermic needle is usually designed to frictionally engage the tip, and possesses certain dimensions which have to be precisely observed in order to assure a perfect fit. For this purpose, the tip surface is not only roughened, but also ground down to such dimensions as to provide for the future thickness of the bi-metallic armor in its finished form. In order to assure perfect interconnections between the two metallic layers, the copper deposit is finished off or polished down and cleansed before the rhodium layer is applied. Upon the completion of the second metallic layer, the latter is finished to the exact dimension required for providing a press fit between the tip and the needle hub.

The edge of the armor adjacent to the uppermost end of the tip, as well as the lower edge of the armor, is carefully trimmed by rolling these edges against the glass, whereby an accurate edge-finish is provided and whereby an intimate contact between glass and metal is established. It is to be noted that upper end 16 of the tip is entirely free of metal and presents an all-glass contacting surface for the interior contacting surface of the hub from which issues the hypodermic needle. Thus, any liquid dispensed by the syringe is not allowed to contact with any metal except that of the needle itself. This can be clearly seen from Fig. 1, where hub 17 is shown in cross-section, and from which extends hypodermic needle 18. It will be also observed from that figure that the interior surface of the hub snugly fits the armor portion surrounding the tip.

In order to illustrate how exactly the armor deposit is to be worked upon the glass, be it assumed that the ultimate dimensions of the tip are to be .319 of an inch at the base of the tip, and .309 of an inch at the end of the tip. The tip has to be ground down at its base to .295 of an inch and at its end to .285 of an inch in order to provide for a .005 of an inch armor coating of the combined metals. Such thickness for small syringes seems to be sufficient to so effectively reinforce the shoulder and tip of the syringe as to prevent breakage for an extended length of use. It is preferred that the armored layers of the two metals be about of the same thickness, that means, .0025" each.

In order to obtain proper accuracy and sufficient density of the relatively soft copper deposit, it is essential that that deposit, particularly at the tip surface, be first made heavier and subsequently worked down to its proper thickness of .0025. A similar procedure is preferably followed when the rhodium layer is deposited, in that a greater thickness of this metal is first allowed to cover the copper, whereupon the surface is gradually reduced to the proper dimension.

In addition to providing the two layers of armor around the tip and the shoulder of the syringe, it is very desirable to re-anneal the syringe and re-glaze the surface of the glass which was formerly roughened, preparatory to the application of the first metal layer. For this purpose the syringe is preferably subjected to an annealing treatment either immediately after the copper layer had been prepared for accommodating the rhodium layer, or upon completion of the bi-metallic armor and after trimming the edges thereof. This procedure assures the elimination

of internal glass strain which may be caused by roughening of the glass surface prior to the plating procedure, and completes the interlocking, through fusing, between the glass and the armor. The foregoing process is applicable to any type 5 of syringe and is not restricted to the syringe described above.

In Fig. 4, there is illustrated the tip end of a glass syringe wherein again a syringe body 10' is shown provided with a shoulder formation 11' and a threaded tip 19, provided with the usual aperture therethrough. It will be observed that the glass portion between the tip and the cylinder is again considerably reduced as to thickness and constitutes the weakest point of the syringe. 15 In this modification, armor 20, consisting of a copper underlayer and a rhodium top layer, is applied to the syringe end in the same manner as described above. It is to be noted that the threads provided in the glass are covered by the 20 armor and are refinished upon completion so as to provide a sharp thread structure.

In the modification shown in Fig. 5, the construction of tip 21 is similar to that shown in Fig. 3, with the exception that the upper portion thereof is made conical while the lower portion 22 is cylindrical and is provided with a small extension 23, adapted to form a bayonet lock between the tip and hub 24 (of Fig. 6), which latter is provided with a bayonet groove 25, for accommodating extension 23. This extension is preferably formed by a drop of glass fused on to the cylindrical portion 22 of the tip, which is subsequently covered by the metallic armor layers. 30

Referring now to Fig. 7, numeral 110 indicates the cylindrical body of a syringe, which is closed by shoulder formation 111, and terminates in a glass tip 112. The closing portion 113 of the glass is again seen to be of considerably lesser thickness than that of the body. Covering the shoulder and tip portions, and extending partially over the shoulder formation along the body, a bi-metallic armor A' is applied in the manner explained previously, with the difference, however, that in this construction the armor, in addition to being united with the pre-prepared glass surfaces by successive electro-deposits and fusing, the metal is positively secured against disengagement by anchoring it in the glass. For this purpose, one or more grooves 26, or other types of depressions are worked into the glass for the reception of relatively heavy metal portions which are caused to fill these depressions and thus veritably anchor the metal in the glass. A similar anchoring effect may be achieved by providing protruding surface-unevennesses, such as the drop of glass shown at 23 in Fig. 5; however, it is preferred to provide grooves, pits or other depressions extending below the glass surfaces to be armored, before or after the same is finished to receive the first metal deposit. 55

In Fig. 7, only a single anchoring groove is illustrated at or near the base of tip 112. It is obvious, however, that a similar groove or depression may be provided at the body surface below the shoulder formation, or that such metal receiving anchoring provision may be located at various other parts of the glass surface to be armored. In this figure, the metal is shown completely filling the groove. It is mechanically practical, and under certain conditions preferable, however, to roll or press the metal deposit into this depression. Such arrangement is not illustrated, since it is quite obvious. 70

## Recapitulation

In each of the above described figures, it will be observed that the glass syringe comprises a cylindrical body, at one end of which there is formed from the glass the shoulder and the tip and that these last named portions of the syringe are continuous and integral parts of the syringe body. It will be also seen that the wall of the shoulder portion is of considerably lesser thickness than that of the cylindrical body of the syringe. The bi-metallic armor deposited upon these weakest points of the syringe are so intimately united with the glass that they form an effective reinforcement, although the thickness of the armor is relatively very thin. Due to this lightness of the armor structure, the syringe does not become top heavy and unwieldy, as is the case with similar devices where the ends are formed with relatively heavy metal fittings.

An important factor of this construction lies in the fact that the contacting surface at the tip end is free of metal and that an all-glass contact is provided for the hub, so that any liquid dispensed by this syringe passes through the passage of the tip directly into the needle.

The fact that the syringe is subjected to a re-annealing treatment is of considerable importance, not only because the strains and stresses in the glass are equalized, but also for the reason that due to the high annealing temperature (of about 900° C.) employed, at least the copper underlayer becomes intimately fused onto the glass. Although we prefer to re-anneal the syringe after the copper is deposited, it is quite satisfactory to subject the syringe to this step of the process after completion of the double armor, and before the armor portion at the tip is worked down to the final dimensions, and before the edges of the armor are trimmed.

While the foregoing invention deals with specific forms and constructions of the devices illustrated, it is quite evident that the same principle of forming an armor upon a glass syringe may be employed in any analogous structures. It is also evident that for various specific purposes the construction of the armor may have to be altered, for which reason we reserve for ourselves the right to make changes and improvements thereon as may become necessary in production, without departing from the broad scope of our invention, as defined in the annexed claims.

We claim:

1. The method of armoring the tip and the shoulder of an annealed glass syringe, which consists of reducing the dimensions of the tip to the extent of the proposed thickness of the armor and roughening the normally glazed surfaces of the tip and of the shoulder, electro-depositing a relatively thick layer of copper on to the roughened surface, re-annealing the syringe and thereby fusing the copper onto the glass, reducing the dimensions of the copper layer at the tip to somewhat below the proposed thickness of the armor, smoothening or polishing and cleansing the entire surfaces of the electro-deposited copper layer, electro-depositing upon the cleansed, polished copper layer a rhodium layer, reducing the armor to its ultimate thickness, and trimming, by rolling-down, the edges of the combined deposits at the end of the tip, so as to provide a clean glass-contacting surface, and at the outer circumference of the shoulder, so as to provide a clean edge.

2. The method of armoring the tip and the shoulder of a glass syringe, as per claim 1, and finishing to fitting dimensions the rhodium deposit at the tip.

3. The method of armoring the tip and the shoulder of a normally annealed glass syringe, which consists of roughening the normally glazed glass surface by grinding down the tip for accommodating the proposed thickness of the armor and etching the surface about the shoulder, electro-depositing first a layer of copper and then a layer of rhodium upon the prepared surfaces to the proposed thickness of the armor, re-annealing the glass, and trimming the edges of the combined deposits by rolling them against the glass, and finishing the rhodium layer at the tip.

4. The combination with the tip and the shoulder of a doubly annealed glass syringe, of an electro-deposited combination armor consisting of an underlayer of copper and a top layer of rhodium, said armor extending to the uppermost edge of the tip, but leaving the glass at the tip end free to provide a non-metallic contacting surface.

5. In a glass syringe, an armored shoulder and tip, the armor extending from the uppermost tip end edge to below the curvature of the shoulder, said armor comprising an electro-deposit of a copper underlayer and a rhodium top layer, the end of the tip providing an all-glass contacting surface, the end edges of the armor being rolled against the glass, for the purpose of providing intimate contact with the glass and for giving the edges a proper trim.

6. In a glass syringe, as per claim 5, and wherein the top layer at the tip is finished to assure perfect fit with the hub of a needle.

7. In a glass syringe, a glass shoulder and glass tip forming continuous and integral parts of the syringe body, the glass at said shoulder being of lesser thickness than that of the body, a bi-metallic armor deposited upon and covering said tip and said shoulder and extending over a portion of the body adjacent to the shoulder formation, said bi-metallic armor consisting of a relatively soft metallic underlayer and a relatively hard metallic upper layer, the tip end being free of the armor to present a clean, all-glass contacting surface, the termini of the armor being rolled against the glass for providing an edge trim, the surface of the armor at the tip being finished to provide perfect fit for a needle hub.

8. In a glass syringe, as per claim 7, and wherein the glass of the syringe is doubly annealed.

9. In a glass syringe, as per claim 7, and wherein the glass of the syringe is doubly annealed and re-glazed.

10. In a glass syringe having a shoulder and a tip, the thickness of the shoulder wall being less than that of the syringe body, a bi-metallic electro-deposited armor fused upon the outer surface of the shoulder and the tip and extending from the uppermost tip edge to somewhat below the shoulder, the termini of the armor being rolled against the glass, the end surface of the tip being bare of metal.

11. The combination with the shoulder and tip of a glass syringe, of a bi-metallic armor fused upon said shoulder and tip and comprising a relatively soft metal underlayer, such as copper, and a relatively hard metal top layer, such as rhodium, and wherein the armored tip is construct-

- ed and arranged for accommodating a corresponding needle hub, and wherein the tip-end is devoid of metal.
12. In an armored glass syringe having a shoulder formation and a tip, a metallic reinforcing armor deposited and fused onto and over the shoulder formation and the tip, and extending partially onto the body of the syringe, means, provided at the glass surface, to which the armor is applied, for anchoring the armor in the glass.
13. In an armored glass syringe, as in claim 12, and wherein said anchoring means constitute a depression extending beneath the main glass surface covered by the armor.
14. In an armored glass syringe, as in claim 12,
- and wherein said anchoring means constitute an annular groove at the base of said tip.
15. The method of reinforcing the shoulder and tip portions of a glass syringe, which consists of roughening the surface of these portions, providing unevenness at the roughened surface, electrodepositing upon the roughened and uneven surface first a relatively soft metal, then a hard metal so that the metals engage said unevenness and form anchoring points for the metal in the glass, subjecting the glass to an annealing temperature, thereby eliminating stresses in the glass and simultaneously fusing the metal onto the glass.

MAX KLEIN.  
GEORGE GRUNBERG.

15